



US006887541B2

(12) **United States Patent**  
Benim et al.

(10) Patent No.: **US 6,887,541 B2**  
(45) Date of Patent: **\*May 3, 2005**

(54) **INSULATED PACKAGING MATERIAL AND POUCH FORMED THEREOF**

(75) Inventors: **Thomas E. Benim**, Goodlettsville, TN (US); **Susan G. Chamberlin**, Wilmington, DE (US); **Jeffrey A. Chambers**, Hockessin, DE (US); **Steven R. Cosentino**, Quinton, VA (US); **Peter R. Hunderup**, Richmond, VA (US); **Ross A. Lee**, Chesapeake City, MD (US); **Susan D. Procaccini**, Hockessin, DE (US); **Donna L. Visiolo**, Lower Gwynedd, PA (US)

(73) Assignee: **E. I. du Pont de Nemours and Company**, Wilmington, DE (US)

(\*) Notice: Subject to any disclaimer, the term of this patent is extended or adjusted under 35 U.S.C. 154(b) by 0 days.

This patent is subject to a terminal disclaimer.

(21) Appl. No.: **10/271,377**

(22) Filed: **Oct. 15, 2002**

(65) **Prior Publication Data**

US 2003/0129335 A1 Jul. 10, 2003

**Related U.S. Application Data**

(63) Continuation-in-part of application No. 09/832,503, filed on Apr. 11, 2001.

(51) **Int. Cl.** <sup>7</sup> ..... **B29D 22/00**

(52) **U.S. Cl.** ..... **428/35.7; 428/202; 428/204; 428/213; 428/215; 428/354; 428/113; 264/495; 264/210.7; 264/173.19; 264/209.5**

(58) **Field of Search** ..... **428/35.7, 202, 428/204, 215, 213, 354, 113; 264/495, 210.7, 173.19, 209.5**

## (56)

**References Cited**

## U.S. PATENT DOCUMENTS

|              |          |                  |
|--------------|----------|------------------|
| 3,401,475 A  | 9/1968   | Morehouse et al. |
| 4,273,816 A  | * 6/1981 | Tollette .....   |
| 4,871,597 A  | 10/1989  | Hobson           |
| 5,164,254 A  | 11/1992  | Todd et al.      |
| 5,404,667 A  | 4/1995   | Schmitter        |
| 5,453,326 A  | 9/1995   | Siddiqui         |
| 5,527,600 A  | 6/1996   | Frankosky et al. |
| 6,150,013 A  | 11/2000  | Balaji et al.    |
| 6,286,872 B2 | * 9/2001 | Barre .....      |
| 6,379,764 B1 | 4/2002   | Pusateri et al.  |

## FOREIGN PATENT DOCUMENTS

|    |                |        |
|----|----------------|--------|
| DE | 130564         | 4/1978 |
| EP | 0101340 A1     | 2/1984 |
| EP | 1064897 A1     | 1/2001 |
| WO | WO 91/04152 A1 | 4/1991 |

## OTHER PUBLICATIONS

www.3M.com, 3M™ Composite Electrical Tape.  
McIntyre, Professor J. E., Daniels, P.N., Editors, Textile Terms and Definitions, 1997, p. 66, p. 351, 10<sup>TH</sup> Edition, The Textile Institute, Biddles Limited, UK.

\* cited by examiner

Primary Examiner—Nasser Ahmad  
Assistant Examiner—Jane Rhee

## (57)

**ABSTRACT**

An insulated packaging material includes a thermal insulating layer, which may a fiberfill batt. The batt is laminated to at least one facing layer of film, paper or fabric. The packaging material can be used as a container, such as a pouch. A food-contacting polymer material is applied to the facing layer to form the inner surface of the pouch. The packaging material may be coated on the outer facing layer with a coating material so that it is printable, thus imparting both insulating properties and print capability to the pouch.

**19 Claims, 8 Drawing Sheets**





FIG. 1



FIG. 2



FIG. 1a



FIG. 1b



FIG. 3



FIG. 4



FIG. 5



FIG. 6



FIG. 7

INSULATED PACKAGING MATERIAL AND  
POUCH FORMED THEREOFCROSS-REFERENCE TO RELATED  
APPLICATION

This application is a continuation-in-part of U.S. patent application Ser. No. 09/832,503, filed Apr. 11, 2001, now pending.

## BACKGROUND OF THE INVENTION

## 1. Field of the Invention

The present invention relates to an insulated packaging material which comprises a thermal insulating layer which is laminated to a face material. The face material may be film, paper or fabric. A polymer sealant material is applied to one surface of the face material. In addition, the face material can be coated with a coating material so that it is printable, thus imparting both insulating properties and print capability to the packaging material.

## 2. Description of Related Art

Insulated enclosures for containers are known, such as that disclosed in U.S. Pat. No. 4,871,597. This enclosure includes a first, or inner-most fabric layer, a second inner-most insulating layer which includes a polymeric foam, a third inner-most metallized polymer film reflective layer, and an outer-most fabric mesh layer. However, the use of four different layers, although providing good insulation for the container, can be cumbersome, which limits the flexibility of the container.

Also known in the film art is a thin electrical tape which comprises a polyester web-reinforced polyester film, as disclosed in 3M Utilities and Telecommunications OEM. However, this tape, which at its thickest is 0.0075 inch (0.0190 cm.), is not suitable for use as an insulated packaging material.

Thus, there exists a need to design an insulated packaging material which is inexpensive to manufacture. Such an insulator would be thick enough to provide adequate insulation, but thin enough to be flexible.

## BRIEF SUMMARY OF THE INVENTION

The present invention overcomes the problems associated with the prior art by providing an insulated packaging material. This insulated packaging material has enough loft, i.e., is thick enough (greater than 0.0075 inch (0.0190 cm)) so as to provide adequate insulation when used, for example, as an insulated pouch, but is thin enough so that it is flexible, for example, as juice pouches are. The insulated packaging material of the present invention is printable, thereby enhancing its use as a packaging material.

Another advantage of the insulated packaging material of the present invention is that it is less costly to manufacture than a typical roller coated or extrusion coated adhesive laminated structure, since in a preferred embodiment it includes a co-extruded film with a heat-sealable adhesive which is used to adhere the film to an insulating layer.

Moreover, in the preferred embodiment where the film and the insulating layer are both made of polyester, and include compatible adhesives, the insulated container stock of the present invention is wholly recyclable, thereby providing significant environmental advantages over known packaging materials of the prior art.

In accordance with the present invention, the insulated packaging material of the present invention comprises a

thermal insulating layer having a thermal resistance of 0.05 to 0.5 CLO (0.0077 to 0.077 m<sup>2</sup>\*K/W) which is laminated to a face material, wherein the insulated packaging material has a thickness in the range of 0.0075 inch (0.0190 cm) and 0.07 inch (0.1778 cm). A polymer film or sealant that is safe for contacting foodstuff is applied to the face material on the surface that will form the interior of an insulated pouch formed from the insulated packaging material.

## BRIEF DESCRIPTION OF THE DRAWINGS

FIG. 1 is a schematic cross-sectional view of an insulated packaging material according to the present invention, showing face material on both sides of a thermal insulating layer.

FIG. 1a is a schematic cross-sectional view of another insulated packaging material according to the present invention, showing face material on both sides of a thermal insulating layer and with a sealant applied to one of the face material layers.

FIG. 1b is a schematic cross-sectional view of yet another insulated packaging material according to the present invention, showing face material on both sides of a thermal insulating layer and with a thicker polymer sealant layer applied to one of the face material layers to enable the insulated packaging material to support a fitment when the material is formed into a pouch.

FIG. 2 is a schematic cross-sectional view of the insulated packaging material of the present invention, similar to FIG. 1, but showing face material laminated to only one side of the thermal insulating layer.

FIG. 3 is a schematic perspective view of a pouch formed from the insulated packaging material.

FIG. 4 is a schematic view of one apparatus suitable for making the label stock or insulated packaging material according to the present invention.

FIG. 5 is graph showing the temperature at which the heat sealable layers of the face material were activated vs. the thickness of the label stock made in Example 1.

FIG. 6 is a graph showing the temperature at which the heat sealable layers of the face material were activated and laminated to the thermal insulating layer vs. thermal insulation values, as measured in CLO, of the label stock made in Example 1.

FIG. 7 is a schematic perspective view of a stand-up pouch with an integral fitment formed from the insulated packaging material.

DETAILED DESCRIPTION OF THE  
INVENTION

In accordance with the present invention, there is provided an insulated packaging material. Such a material is shown generally at 5 in FIGS. 1 and 2 and rolled up at 220 in FIG. 4. The packaging material is cut into individual lengths to make packages, such as pouches, a sample of which is illustrated in FIG. 3.

The insulated packaging material of the present invention includes a thermal insulating layer shown at 30 in FIGS. 1 and 2. This thermal insulating layer has a thermal resistance as measured in units of insulation, or CLO, of 0.05 to 0.5. The CLO unit is defined as a unit of thermal resistance of a garment. The SI unit of thermal resistance is the square-meter kelvin per watt (m<sup>2</sup>\*K/W) (See "Textile Terms and Definitions", Tenth Edition, The Textile Institute, (1995). pp. 66, 350). Thus, the range of thermal resistance in SI units of the thermal insulating layer of the present invention is

0.0077 to 0.077 m<sup>2</sup>\*K/W. Although CLO is defined in terms of a garment, this measurement can be used to describe the thermal resistance of any textile system, and is used herein to describe the thermal resistance of the thermal insulating layer of the present invention. CLO values depend on the material used for the insulating layer and its thickness. CLO values of labels made without the thermal insulating layer of the present invention were below the lower end of the range (0.05 CLO, or 0.0077 m<sup>2</sup>\*K/W).

The thermal insulating layer comprises an organic thermoplastic fiber based material comprising polyester, polyethylene or polypropylene. In a preferred embodiment, the thermal insulating layer is a fiberfill batt comprising polyester. A fiberfill batt sold as THERMOLITE® Active Original by E. I. du Pont de Nemours and Company is especially suitable for use with the present invention. The fiberfill batt used with the present invention has an areal weight in the range of 10 gm/m<sup>2</sup> to 200 gm/m<sup>2</sup>, and a bulk density of less than 0.3 gm/cm<sup>3</sup>. Alternatively, the thermal insulating layer may comprise melt blown fibers, such as melt blown polyolefins, sold as THINSULATE®, by 3M.

Many other variations of insulating material for the thermal insulating layer can be used with the present invention. For instance, the thermal insulating layer may comprise a foam. The foam may be polyurethane or polypropylene, or any other foam composition as known in the art. Or the thermal insulating layer may be made of an inorganic thermoplastic fiber based material comprising glass wool, borosilicate glass or rockwool.

Alternatively, the thermal insulating layer may comprise a knit fabric, made, for example from a tetrachannel or scalloped oval fiber, sold under the trademark COOLMAX® by E. I. du Pont de Nemours and Company of Wilmington, Del. Or the thermal insulating layer may be a woven or fleece material. The insulating layer could also comprise some sort of nonwoven, such as felt, or a highloft nonwoven or needled nonwoven fabric.

The thermal insulating layer is laminated to a face material, shown at **10** in FIGS. 1 and 2 and also at **20** in FIG. 1. By "lamination" is meant uniting layers of material by an adhesive or other means. The face material may be film, paper and/or fabric. The film is made of a thermoplastic material comprising either polyester, polyethylene or polypropylene. In the embodiment illustrated in FIG. 1, the thermal insulating layer is laminated between two sheets of film, paper or fabric. However, it is within the scope of the present invention to laminate a single sheet of face material to the thermal insulating layer, as shown in FIG. 2. The use of a single sheet of face material will not affect the thickness of the packaging material substantially, since the thickness of the face material is insignificant compared to the total thickness of the packaging material. The packaging material of the present invention is greater than 0.0075 inch (0.0190 cm.) thick, so that it is thick enough to provide adequate insulation for a package. However, the packaging material should be thin enough to be flexible, and should be preferably less than 0.07 inch (0.1778 cm). Face material **10**, including first layer **13** and second **14** layer as shown in FIGS. 1 and 2 and face material **20**, including first layer **22** and second layer **24** as shown in FIG. 1 may be of thickness between 0.0002 inch (0.0005 cm) and 0.010 inch (0.025 cm). A preferred range for the thickness of the face material is 0.00048 inch (0.00121 cm) to 0.0020 inch (0.0050 cm).

In a preferred embodiment, hereinafter referred to as the "co-extruded film" embodiment, the face material comprises a film which is co-extruded so that it comprises two layers.

Thus, face material **10** comprises a first layer **13** and a second layer **14**. In this embodiment, first layer **13** and second layer **14** are made of different materials, but form one sheet of film. Second layer **14** is heat sealable—i.e., it is made of a material which has a lower melting temperature than the material of first layer **13**, so that when face material **10** is heated, second layer **14** softens and adheres to the thermal insulating layer when pressure is applied. Similarly, face material **20** comprises a first layer **22** and a second layer **24**. Again, first layer **22** and second layer **24** are made of different materials, but form one sheet of film. Second layer **24** is heat sealable—i.e., it is made of a material which has a lower melting temperature than the material of first layer **22**, so that when face material **20** is heated, second layer **24** softens and adheres to the thermal insulating layer when pressure is applied.

Alternatively, rather than "co-extrusion", layers **13** and **14** and **22** and **24** may be formed by coating separate layers of polymer solution onto the surfaces of the thermal insulation layer.

As shown in FIG. 1a, a sealing material **62** or polymer sealant layer that is safe for contacting foodstuff that may be stored within the pouch formed from the insulating packaging material is applied to the face material. The sealing material **62** preferably comprises a layer of one or more polymers, such as a polyester copolymer, poly(vinylidene chloride), or a copolymer of ethylene with vinyl acetate. The sealing material may be applied directly to the facing material (often polyester) sheet after the sheet has been extruded, and either before or after the sheet is oriented. The polymer sealant layer preferably has a thickness in the range of 0.0025 mil to 5 mil (6.35×10<sup>-6</sup> cm to 0.0127 cm). It may be applied to the face material as a co-extruded web structure, optionally with an oxygen barrier. If the co-extruded web structure has an oxygen barrier, the web structure preferably includes in addition to the sealant layer an oxygen barrier layer material, such as poly(vinylidene chloride) or ethylene-vinyl alcohol (EVOH).

Referring to FIG. 1b, sealing material **62a** may be a polyethylene or ethylene copolymer having a thickness greater than the sealing material **62** in FIG. 1a. The thickness of sealing material **62a** is in the range of 0.005 mil to 5 mil (12.7×10<sup>-6</sup> cm to 0.0127 cm) to enable attachment of a fitment **314** to the pouch **310** shown in FIG. 7.

The packaging material of the present invention can further include a coating on the face material. The coating, shown at **12** in FIGS. 1 and 2, is provided on the non-heat sealable surface (i.e., first layers **13** and **22**) of the face material. This coating is printable, so that the packaging material may also function as a label. The coating is a standard print primer based on aqueous polymer dispersions, emulsions or solutions of acrylic, urethane, polyester or other resins well known in the art. (See, for example, U.S. Pat. No. 5,453,326). Alternatively, if the thermal insulating layer is previously printed, and the face material is clear, the need for coating the face material to make it printable may be eliminated.

In a preferred configuration of the co-extruded film embodiment, films with two different thicknesses are used for the face materials, such as face material **10** and face material **20** in FIG. 1. One specific example of a film which is suitable for use as face material **10** in FIG. 1 is **4 MELINEX® 854**, commercially available from DuPont Teijin Films of Wilmington, Delaware. **MELINEX® 854** is a 120 gauge (0.0012 inch, or 0.0030 cm.) thick co-extruded biaxially oriented polyester film. The first layer of this film,

such as 13 in FIG. 1, is made from a standard polyester homopolymer, intrinsic viscosity of about 0.590, containing 2500 ppm inorganic slip additive particles. This layer comprises approximately 65% of the total film thickness. A co-polyester resin comprised of 18 weight % isophthalic acid, intrinsic viscosity of about 0.635, containing 2300 ppm inorganic slip additive particles, is co-extruded to form the heat sealable layer (such as 14 in FIG. 1) and comprises 35% of the total film thickness (15–40% preferred). The surface of the first layer opposite the heat sealable layer is coated in-line by a gravure coater (during the film manufacturing process) with a print primer coating (12 in FIG. 1) based on an aqueous polyester dispersion described earlier at a dry coat-weight of 0.03 g/m<sup>2</sup>. MELINEX® 854 film is also suitable for use as face material 20 in FIG. 1, but this face material is slightly thinner than the face material used as face material 10. In all other aspects, the MELINEX® 854 film used as face material 20 is the same as the MELINEX® 854 film used as face material 10 described above.

According to another aspect of the present invention, the face material may be modified on the surface facing away from the thermal insulating layer to facilitate printing thereon by a corona discharge treatment. Specifically, the surface of first layer 13 or 22 is modified. The corona discharge treatment may be done in addition to, or in lieu of, the coating on the face material. Or, alternatively, on top of the coating, or instead of the coating, a vapor deposited metal layer, such as an aluminum layer, may be deposited on the surface facing away from the thermal insulating layer for decorative purposes and for adding optical effects. If this vapor deposition is done, then corona discharge treatment would typically not be performed in addition to this vapor deposition.

According to another modification of the present invention, the face material may be embossed on the surface facing away from the thermal insulating layer in such patterns as may be desired for decoration. The embossing can be done on top of the coating, after corona discharge treatment, if required, and on top of the vapor deposition. Specifically, pressure and heat may be used to make certain areas of the face material thinner, so that the surface appears raised from the areas which were made thinner. Doing so in a pattern may be used to ornament the packaging material. The heat and pressure may be applied by a shaped anvil or iron in a decorative pattern. Alternatively, heat and pressure may be applied by an engraved or etched embossing roller or an engraved reciprocating die in a platen press. The heat should be applied at 200–400° F. (93–204° C.), so that the pressure applied would create permanent indentations in the packaging material. The heat should be applied as to soften at least the face material, and perhaps also the thermal insulating layer. Softening the thermal insulating layer is less critical than softening the face material, but helps the embossing process also.

In addition, the surface modification (i.e., the coating or the corona discharge treatment) may be used to facilitate bonding to another surface with an adhesive layer. In order to bond to another surface, an adhesive Layer, such as that shown at 26 in FIG. 1, is applied to the untreated surface of the face material or to the corona discharge treated surface (but not to a vapor deposition modified or embossed surface). This adhesive layer is pressure sensitive to enable application of the label to a container. In addition, a release liner 28 may be provided on the surface of adhesive layer 26 as shown in FIG. 1. The function of the release liner is to protect the adhesive until the point of application of the label to a container.

The packaging material of the present invention may be sealed, such as with a hot knife, at its edges so that fluid cannot penetrate the edges of the label stock. Alternatively, the packaging material may be self-sealing. In this self-sealing configuration, the packaging material may be folded back onto itself, so that the top and bottom edges are already sealed. A package or pouch made from the packaging material of the present invention is preferably sealed so that fluid cannot penetrate the edges thereof.

10 Further in accordance with the present invention, there is provided an insulated pouch 300. Such a pouch 300 is shown generally in FIG. 3. The insulated packaging material 5 is formed into pouch 300, by sealing the peripheral edges 302, preferably by heating. Various form-fill-seal pouching machines or stand-up pouch forming machines for forming pouches suitable for holding foodstuff and liquids are known in the art, such as an Emzo® EV1 vertical liquid pouch packaging machine available from Emzo Corp., formerly of Argentina, or a Bartelt IM offered by Klockner Bartelt of Sarasota, Fla., USA, or a Toyo Model MS offered by Toyo Machine Mfg. Co. of Nagoya, Japan. Generally, under applied compression pressure and heat, such as by a heat bar in pouch making equipment, the polymer sealant material softens and adheres together to form the sealed peripheral edge.

20 In one region of the pouch, a frangible seal 304 portion is formed along the outer periphery. The frangible seal ruptures more easily than the other sealed regions. For example, the 30 frangible portion 304 will break or separate when heated to the softening point or melting point of the sealant material forming the frangible portion. The portion 304 of the sealed peripheral edge of the pouch may be made frangible by heat sealing this portion at a lower temperature or pressure. Alternatively, one or more frangible seals may be incorporated within the volume of the pouch to create separate compartments (not shown) that keep apart foodstuffs within the pouch until the frangible seals rupture upon heating or upon applied pressure.

30 The temperature at which the frangible portion 304 separates or ruptures varies according to the material selected. In one embodiment, the frangible seal ruptures when the temperature inside the container or pouch exceeds the lower melting point sealant's melting point or softening point. For the polymers used in the facing material of the instant insulated packaging material, the frangible seals generally rupture when the temperature inside the container or pouch formed from the material exceeds 100° C. (212° F.).

40 A frangible target 306 or access port for accessing the pouch volume with a straw also may be provided on one side 45 surface of the pouch 300.

A preferred pouch is formed as a stand up pouch 310 as shown in FIG. 7, which has a gusset 316 in the bottom that when spread apart by the contents of the pouch, allows the pouch 310 to repose vertically without external support. The pouch 310 is formed by folding and sealing the insulating packaging material such as shown in FIG. 1b at the peripheral edges 312 in stand-up pouch forming equipment.

45 After the pouch 310 is formed, a fitment 314 is installed into a surface of the pouch or at its periphery. As shown in FIG. 7, the fitment 314 comprises a tube with screw threads about its outer circumference and an associated threaded cap that can be attached thereto. Examples of such fitments are available from Menshen USA of Waldwick, N.J. The neck of the fitment is held in place at the sealed edge of the pouch either by the sealed edge or by added caulking. Most commonly, the fitment is made of a material that can be heat

sealed onto the facing material or polymer sealant layer forming the inner surface of a pouch. The neck or base of the fitment is then welded into the open end of the pouch by heat sealing between heated jaws or other polymer welding technique. Other fitments used to close and seal containers for vacuum packing and/or holding foodstuffs are also embraced generally within the term "fitment" as used herein, including a zipper closure formed with polymer materials, and a plug.

Further in accordance with the present invention, there is provided a method for making an insulated packaging material. This method is illustrated with reference to FIG. 4. In this method, a sheet of material used for the thermal insulating layer, such as fiberfill batt 30, is fed from a supply roll 45. In addition, face material 10 is fed from a supply roll 40 and is disposed such that coating 12 is oriented away from thermal insulating layer 30 and second layer 14 is facing thermal insulating layer 30. In addition, face material 20 may be fed from a supply roll 50 and is disposed such that the adhesive layer (if required, such being shown at 26 in FIG. 1) is oriented away from the thermal insulating layer. The first layer, such as 13 as shown in FIGS. 1 and 2 and 22 as shown in FIG. 1, of the face material is oriented away from the thermal insulating layer, and the second layer of the face material, such as 14 in FIGS. 1 and 2 and 24 as shown in FIG. 1, faces the thermal insulating layer.

A sheet of the thermal insulating layer, such as 30, and at least one sheet of face material, such as 10 are fed into a heated calender roll nip between a pair of heated calender rolls 70 and 80, shown in FIG. 4. The heated calender rolls cause the surfaces of the thermal insulating layer and the face material to adhere to each other. The calender rolls are heated to a temperature which activates the heat-sealable layer but which does not melt the entire face material as discussed above. This temperature is in the range of 200° F. to 500° F. (93° C. to 260° C.), with the preferred temperature range being 280°–320° F. (137°–160° C.) for the embodiment using co-extruded 48 gauge and 120 gauge films as the face material and a fiberfill batt as the insulating layer. However, higher temperatures in the range of 450°–500° F. (232°–260° C.) can be used at high line speeds, i.e., speeds of 300 to 400 feet (91 to 122 meters) per minute. The calender rolls are displaced from one another at a distance appropriate to create a nip pressure suitable for lamination.

Alternatively, instead of using a coextruded heat sealable film, an adhesive may be applied between the face material and the thermal insulating layer to adhere them together. This adhesive would be applied by a coating roller, not shown, which would be positioned between feed rolls 40 and 50 and calender rolls 70 and 80 in FIG. 4. A packaging material is formed which is pulled through the process equipment by means of a take-up roll 220 as shown in FIG. 4.

A packaging material with a thickness of greater than 0.0075 inch (0.0190 cm.) but less than 0.07 inch (0.1778 cm), preferably between 0.010 inch (0.025 cm.) and 0.040 inch (0.102 cm.), and most preferably between 0.020 inch (0.051 cm.) and 0.030 inch (0.076 cm.) is thus produced. This packaging material could be made with one sheet of face material, as in FIG. 2, or two sheets of face material, as in FIG. 1, since the thickness of the face material is insignificant compared to the total thickness of the material. The formation of the packaging material may be followed by cutting to desired widths with a hot knife which seals the edges. The packaging material may then be cut to form pouches, which may preferably have sealed edges.

Alternatively, instead of using a single sheet of face material, the thermal insulating layer may be fed between

two sheets of face material into the heated calender roll, which causes the surfaces of the thermal insulating layer and the face material to adhere to each other. This embodiment is also illustrated in FIG. 4, where both face materials 10 and 20 are fed to the nip between heated calender rolls 70 and 80. In either embodiment where either one or two sheets of face material are fed between heated calender rolls, the thermal insulating layer batt may be previously printed, thereby eliminating the need for coating the face material to make it 10 printable.

It should be apparent to those skilled in the art that modifications may be made to the method of the present invention without departing from the spirit thereof. For instance, the present invention may alternatively include a 15 method for making an insulated packaging material, wherein a card web comprising thermoplastic staple fibers is fed from a commercially available card machine. This card web is run in place of the fiberfill batt in the process described above with respect to FIG. 4, thereby being deposited 20 directly onto a face material. The card web and face material are subjected to a calendering process, thereby laminating the fibers from the card web to the face material. It should be noted that the packaging material made in accordance with this embodiment is by design thinner than the preferred 25 embodiment thickness, which is between 0.020 inch (0.051 cm.) and 0.030 inch (0.076 cm.), but still would be greater than 0.0075 inch (0.0190 cm.).

The present invention will be illustrated by the following 30 Examples. The test method used in the Examples is described below.

#### TEST METHOD

For the following Examples, CLO was measured on a 35 "Thermolabo II", which is an instrument with a refrigerated bath, commercially available from Kato Tekko Co. L.T.D., of Kato Japan, and the bath is available from Allied Fisher Scientific of Pittsburgh, Pa. Lab conditions were 21° C. and 65% relative humidity. The sample was a one-piece sample 40 measuring 10.5 cm×10.5 cm.

The thickness of the sample (in inches) at 6 gm/cm<sup>2</sup> was determined using a Frazier Compressometer, commercially 45 available from Frazier Precision Instrument Company, Inc. of Gaithersburg, Md. To measure thickness at 6 g/cm<sup>2</sup>, the following formula was used to set PSI (pounds per square inch) (kilograms per square centimeter) on the dial:

$$\frac{(6.4516 \text{ cm}^2/\text{in}^2)(6 \text{ g}/\text{cm}^2)}{453.6 \text{ g}} = 0.8532 \text{ lb/in}^2$$

A reading of 0.8532 on the Frazier Compressometer Calibration Chart (1 in., or 2.54 cm. diameter presser foot) shows that by setting the top dial to 3.5 psi (0.2 kilograms per 55 square centimeter), thickness at 6 g/cm<sup>2</sup> was measured.

The Thermolabo II instrument was then calibrated. The temperature sensor box (BT box) was then set to 10° C. above room temperature. The BT box measured 3.3 inch×3.3 inch (8.4 cm×8.4 cm). A heat plate measuring 2 inch×2 inch was in the center of the box, and was surrounded by styrofoam. Room temperature water was circulated through a metal water box to maintain a constant temperature. A sample was placed on the water box, and the BT box was placed on the sample. The amount of energy (in watts) 60 required for the BT box to maintain its temperature for one minute was recorded. The sample was tested three times, and the following calculations were performed:

$$\text{Heat Conductivity (W/cm}^{\circ}\text{C.}) = \frac{(W)(D \times 2.54)}{(A)(\Delta T)}$$

Where:

W=Watts

D=Thickness of sample measured in inches at 6 g/cm<sup>2</sup>. (6 g/cm<sup>2</sup> was used because the weight of the BT box is 150 gm, the area of the heat plate on the BT box was 25 cm<sup>2</sup>). Multiplying the thickness by 2.54 converted it to centimeters.

A=Area of BT Plate (25 cm)

ΔT=10° C.

$$CLO = \frac{\text{Thickness} \times 0.00164}{\text{Heat Conductivity}}$$

The value of 0.00164 was a combined factor including the correction of 2.54 (correcting thickness from inches to centimeters) times the correction factor of 0.0006461 to convert thermal resistance in cm<sup>2</sup>×° C./Watts. To convert heat conductivity to resistance, conductivity was put in the denominator of the equation.

#### Example 1

A label stock was made according to the process described above with respect to FIG. 4, except that instead of feeding face materials 10 and 20 from supply rolls, they were fed as individual sheets to the nip. The label stock was cut to a length to form a label. A fiberfill batt of the type sold by E. I. DuPont de Nemours and Company of Wilmington, Del. under the trademark THERMOLITE® Active Original was used as the thermal insulating layer. The fiberfill batt had an areal weight of 100 gm/m<sup>2</sup> at a specified thickness of 0.25 inch (0.63 cm), or a bulk density of 0.013 gm/cm<sup>3</sup>.

The films used as the face material were of the type sold by DuPont Teijin Films of Wilmington, Del. under the trademark MELINEX® 301-H. (This film was the same film as MELINEX® 854 as described above, but it did not include the primer coating, such as 12 and 26 as shown in FIG. 1). The composition of the heat-sealable layers (e.g., 14 and 24 in FIG. 1) was an isophthalic acid-based copolyester and comprised 10–50% of the total film thickness; 15–30% was preferred. In this embodiment, face material 10 was 1.2 mils (0.0012 inch, or 0.0030 cm) thick and face material 20 was 0.48 mils (0.00048 inch, or 0.00122 cm) thick. The final label stock thickness, after lamination, was 0.025 inch (0.064 cm). A label was made from this label stock which was wrapped around a can. Another label was made from this label stock which was wrapped around a blown polyester bottle.

The heat sealable layers were activated at temperatures between 240 and 350° F. (116–177° C.). The data is shown in TABLE 1 below, and is graphed in FIGS. 5 and 6. As can be seen from FIGS. 5 and 6, the effect of using different activation temperatures is to give greater thickness and greater insulation value at the lower temperatures, and less thickness and lower insulation values at the higher temperatures.

TABLE 1

| 5  | Temp<br>(° F.) (° C.) | Thickness<br>(in)(cm) | Thermal Resistance<br>CLO (m <sup>2</sup> · K/W) |
|----|-----------------------|-----------------------|--------------------------------------------------|
|    | 240 (115)             | 0.041 (0.104)         | 0.272 (0.042)                                    |
|    | 250 (121)             | 0.036 (0.091)         | 0.226 (0.035)                                    |
|    | 280 (138)             | 0.03 (0.076)          | 0.199 (0.030)                                    |
| 10 | 310 (154)             | 0.027 (0.069)         | 0.17 (0.026)                                     |
|    | 350 (177)             | 0.024 (0.061)         | 0.141 (0.021)                                    |

#### Example 2

An insulated pouch was made according to the process described above with respect to FIG. 4. A fiberfill batt of the type sold by E. I. du Pont de Nemours and Company of Wilmington, Del. under the trademark THERMOLITE® Active Original was used as the thermal insulating layer. The fiberfill batt had an areal weight of 100 gm/m<sup>2</sup> at a specified thickness of 0.25 inch (0.63 cm), or a bulk density of 0.013 gm/cm<sup>3</sup>.

The pouches were made by combining a roll of polyester film laminated to a polyolefin with a roll of film composed of two layers of polyester film having a layer of thermal insulator between them.

The films used as the face material were of the type sold by DuPont Teijin Films of Wilmington, Del. under the trademark MELINEX® 854. The composition of the heat-sealable layers was an isophthalic acid-based copolyester and comprised 10–50% of the total film thickness; 15–30% was preferred. The MELINEX® film was laminated to a polyethylene film of the type sold by Nova Chemicals under the trademark SCLAIR® SL-1 using a solution-based adhesive of the type sold by Rohm and Haas Co. of Philadelphia, Pa. under the trademark MORTON 503A. The adhesive was applied by a 110 Quad gravure roll with a doctor blade. The films were combined in the nip roll at 190° F. (87.8° C.) and coated at a speed of 25 feet per minute, then the laminated film was dried at 160° F. (71.1° C.). The roll containing the thermal insulator was composed of 1.2 mil MELINEX® 854, THERMOLITE® Active Original, and 0.48 mil MELINEX® 854 by DuPont Teijin films and was prepared by laminating the layers in the same way described above.

A pouch was made from this insulated packaging stock using the EMZO® EV1 vertical liquid pouch packaging machine available from Emzo Corp., formerly of Argentina. Alternate pouch making equipment includes the Bartelt IM offered by Klockner Bartelt of Sarasota, Fla., USA and the Toyo Model MS offered by Toyo Machine Mfg. Co. of Nagoya, Japan.

The rollstock was fed into the pouch packaging machine and was heat sealed on four sides and cut to desired dimensions to form pillow pouches. The heat sealable layers were activated at a seal temperature of 200° C. (392° F.). Pouches were produced at a rate of 40 pouches per minute.

What is claimed is:

1. An insulated packaging material, comprising:  
a sheet of face material formed as a bi-layer film having a first layer and a second layer, wherein said second layer has a lower melting temperature than said first layer;  
a polymer sealant layer applied to the first layer of the sheet; and  
a thermal insulating layer comprising one or more materials selected from the group consisting of fiberfill batt, melt blown fibers, knit fabric, woven material, and

**11**

fleece; the thermal insulating layer having a thermal resistance in the range of 0.05 to 0.5 CLO (0.0077 to 0.077 m<sup>2</sup>\*K/W) laminated to the second layer of the sheet, to form the packaging material having a thickness in the range of 0.0075 inch (0.0190 cm) to 0.07 inch (0.1778 cm).<sup>5</sup>

2. The insulating packaging material of claim 1, wherein the polymer sealant layer is selected from the group consisting of polyethylene, polyester, and copolymers thereof.

3. The insulating packaging material of claim 1, wherein the polymer sealant layer is applied to the face material as a coextruded web structure.<sup>10</sup>

4. The insulating packaging material of claim 1, further comprising a second sheet of face material formed as a bi-layer film having a first layer and a second layer, wherein said second layer has a lower melting temperature than said first layer, wherein said second sheet is laminated to the thermal insulating layer.<sup>15</sup>

5. The insulating packaging material of claim 1, further comprising a printable coating on the second sheet of face material.<sup>20</sup>

6. An insulated pouch made of the insulated packaging material of claim 1.

7. The insulated pouch of claim 6, wherein the pouch defines a storage volume, and further comprising a fitment that facilitates access to the storage volume.<sup>25</sup>

8. The insulated pouch of claim 6, wherein the pouch defines a storage volume, and further comprising a zipper that facilitates access to the storage volume.

9. The insulated pouch of claim 6, further including a frangible sealing surface.<sup>30</sup>

10. A method for making an insulated packaging material as recited in claim 1, comprising:

providing a sheet of face material formed as a co-extruded film having a first layer and a second layer, wherein said second layer has a lower melting temperature than said first layer;<sup>35</sup>

applying a polymer sealant layer to the first layer of the sheet to produce a sheet with the applied polymer sealant; and

**12**

feeding the sheet with the applied polymer sealant and a thermal insulating layer having a thermal resistance in the range of 0.05 to 0.5 CLO (0.0077 to 0.077 m<sup>2</sup>\*K/W) into a calender roll nip to cause the sheet and thermal insulating layer to be laminated together wherein the thermal insulating layer is laminated to the second layer of the sheet, to form the packaging material having a thickness in the range of 0.0075 inch (0.0190 cm.) and 0.07 ((0.1778 cm).<sup>5</sup>

11. The method of claim 10, wherein the polymer sealant layer is selected from the group consisting of polyethylene, polyester, and copolymers thereof.

12. The method of claim 10, wherein the polymer sealant layer is applied to the face material as a coextruded web structure.<sup>10</sup>

13. The method of claim 10, further comprising laminating to the thermal insulating layer a second sheet of face material formed as a co-extruded film having a first layer and a second layer, wherein said second layer has a lower melting temperature than said first layer.<sup>15</sup>

14. The method of claim 13, further comprising applying a printable coating onto the second sheet of face material.<sup>20</sup>

15. The method of claim 10, further comprising sealing together edges of the insulated packaging material to form a pouch.<sup>25</sup>

16. The method of claim 15, further comprising installing a fitment in the pouch.<sup>30</sup>

17. The method of claim 15, further comprising sealing a portion of one edge of the pouch with a sealant having a lower melting point to form a frangible seal.<sup>35</sup>

18. The method of claim 17, wherein the frangible seal is formed so as to rupture when the temperature inside a volume defined by the pouch exceeds 100° C.

19. The insulated packaging material of claim 1, wherein the thermal insulating layer comprises fiberfill batt.

\* \* \* \* \*